

Oct. 21, 1930.

G. O. SMALL

1,779,295

METHOD OF MANUFACTURING NONMETALLIC GEAR WHEELS AND THE LIKE

Filed April 18, 1928

Fig. 1.



Fig. 2.



Fig. 3.



Fig. 4.



Inventor:  
Guy O. Small,  
by *Charles E. Muller*  
His Attorney.

## UNITED STATES PATENT OFFICE

GUY O. SMALL, OF LYNN, MASSACHUSETTS, ASSIGNOR TO GENERAL ELECTRIC COMPANY, A CORPORATION OF NEW YORK

## METHOD OF MANUFACTURING NONMETALLIC GEAR WHEELS AND THE LIKE

Application filed April 18, 1928. Serial No. 270,995.

The present invention relates to non-metallic gear wheels or the like, of the type comprising spinnable textile fibers held under high compression between metal end 5 plates, and especially to such gear wheels or the like formed from cotton fibers and wherein the gear wheel or the like is formed by cutting disks from sheets of cotton material, stacking the disks one on another between 10 metal end plates and then compressing the stack and fastening the end plates together with studs or other suitable means. The invention relates especially to the manufacture of such gear wheels from unwoven cotton 15 ton fibers although it is not limited thereto necessarily.

In manufacturing gear wheels or the like from loose cotton fibers, it is desirable in the first instance to consolidate layers of the 20 fibers into sheets which are sufficiently stiff and board-like to enable them to be handled readily and to have blanks cut from them. Heretofore, as far as I am aware, this has been accomplished by first immersing cotton 25 batting or similar unwoven sheet cotton in a solution of water and starch and afterwards pressing and drying the material, there being thus obtained board-like sheets sufficiently stiff to be handled and to have cut 30 therefrom readily disks for forming the gear wheels or the like. This method, while satisfactory, has the disadvantage that it adds to the cotton fibers a certain amount of starch which, while not harmful, is not 35 essential to the finished product and that it requires careful drying to remove all the water from the cotton fibers, it being the practice to subject the structure after it has been finally compressed between the end 40 plates to a vacuum treatment to remove the last trace of water and then to admit oil to the vacuum chamber in which the treatment is taking place so as to fill the interstices in the compressed cotton with oil which 45 serves as a lubricant and also as a means to prevent the structure afterwards from absorbing moisture. Also, this method of treating the cotton batting with a starch solution has the disadvantage that it renders 50 the waste left from cutting disks from the

sheets unfit to be re-worked and again used in the process. And in addition to the foregoing, this former method has the disadvantage that it comprises a number of steps and requires the use of a relatively expensive 55 form of cotton fibers, i. e. cotton batting, which means that the method is relatively expensive.

The object of my invention is to provide an improved method of manufacturing gear 60 wheels, gear wheel blanks or the like from loose cotton fibers which is simpler than methods heretofore in use, and whereby I am enabled to reduce materially the cost of manufacture and at the same time increase 65 the strength of the gear wheel.

For a consideration of what I believe to be novel and my invention, attention is directed to the accompanying description and the 70 claims appended thereto.

According to my invention, I take spinnable textile material which may be in the form of loose, unwoven cotton such as a picker lap or cotton batting, for example, or which may be in the form of woven material 75 and treat it with a small amount of lubricating oil, very light machine oil being satisfactory, and following this, I then press the oil-treated material between heated rolls or in a suitably heated press. I have found that by this means I am enabled to provide a board-like sheet of cotton material which is sufficiently stiff to be handled readily and from which disks can be cut and utilized in a known way for the manufacture of gear 80 wheels, gear wheel blanks or the like. 85

The material is treated with just sufficient oil that during the final consolidation of the structure, little if any oil will be squeezed out. At the same time, however, sufficient oil is 90 used so that if the final structure were subjected to an oil solution in a vacuum, no more oil would be taken up by the fibers of the material. The oil may be applied to the material in any suitable manner, the only essential being that it be distributed fairly uniformly over the material. In compressing the oil-treated material in the case of cotton material, a pressure of the order of 1000 lbs. per sq. in. is satisfactory, the material be- 95 100

ing at the same time subjected to a temperature of the order of 325° F.

Broadly considered, my improved method comprises first treating the material such as loose cotton fibers with a suitable amount of oil; then compressing the oil-treated material to form board-like sheets which are sufficiently stiff to be handled readily; and finally, in a manner already known, cutting disks from the sheets, stacking the disks between metal end plates, compressing the stack under high pressure, and fastening the end plates together by means of studs or other fastening means. My invention comprises also an improved method whereby I am enabled to utilize advantageously baled cotton which can be purchased at relatively low cost as compared with cotton batting, for example.

In the drawing, I have illustrated apparatus by which my invention may be carried out with advantage, the apparatus enabling me to utilize baled cotton, a form in which the cotton can be purchased at relatively low cost.

In the drawing, Figs. 1 and 2 are diagrammatic views illustrating in a general way apparatus which may be utilized in carrying out my invention; Fig. 3 is a perspective view of a sheet of material as it comes from the apparatus illustrated in Figs. 1 and 2; Fig. 4 shows the manner in which the material is stacked to form a gear wheel blank, and Fig. 5 shows a completed gear wheel blank.

Referring to the drawing, Fig. 1, 6 indicates diagrammatically a two beater breaker and picker. This may be of any desired type, such machines being known in connection with the working of textile materials such as raw cotton. It comprises generally a hopper in which a bale of cotton comber waste or card strips may be placed and mechanism which serves to separate the cotton fibers, clean them and spread them out into a relatively thin sheet. The sheet of cotton fibers leaving the two beater breaker and picker 6 is indicated at 7. It passes between sets of rollers 8 and 9, and is finally wound into a roll by the rollers 10 as is indicated at 11. Prior to being formed into roll 11, the sheet of cotton fibers is sprayed with a small amount of lubricating oil such, for example, as a very light machine oil. This oil may be sprayed on in any suitable manner. In the present instance it is shown as being sprayed by means of a revolving brush 12 which engages the surface of a revolving metal cylinder 13 the lower portion of which dips into a receptacle 14 containing the lubricating oil. A certain amount of oil is carried up on the surface of the metal cylinder and is brushed off by the revolving brush 12 and deposited on the cotton sheet. The spray of oil is indicated at 15. A number of rolls 11 of suitable size may be formed, each roll being wound on an arbor 16.

Referring now to Fig. 2, a number of the rolls 11 of oil treated fibers are placed in a

framework comprising pairs of vertical arms 17 slotted as is indicated at 18 to receive arbors 16. 19 is an endless belt which is caused to travel by the rollers 20, the belt being located just beneath the lower edges of slots 18. A number of the rolls 11 are arranged in the slots 18 as shown in Fig. 2, each one being unrolled slightly so that the ends of the successive rolls are in engagement with each other. The friction between the belt and the sheets of the cotton fiber is such that as the belt 19 travels the rolls 11 are unrolled forming thereby a relatively thick sheet of loose cotton fibers, as is indicated at 21. This sheet is fed through pairs of heated pressure rolls 22 which serve to heat and compress it. I have found that by this treatment there is obtained a board-like sheet of cotton fibers which is sufficiently stiff to be handled readily and to have blanks cut from it. 23 indicates a suitable cutting tool which may be utilized for cutting the board-like sheets into lengths of convenient size.

Fig. 3 indicates at 24 one of the sheets which has been cut off by the tool 23. From the sheet 24 discs of suitable size, as is indicated at 25 in Fig. 4, may be cut. These discs are stacked one on top of another between suitable metal end plates after which the entire structure is consolidated in a suitable hydraulic press and fastened in compressed condition to form a gear-wheel blank or the like.

Fig. 5 indicates a completed gear-wheel, 26 indicating the layers of cotton fiber, 27 the metal end plates, 28 studs which serve to hold the structure assembled, and 29 teeth which have been cut in the blank.

By my invention I have materially simplified the method of manufacturing non-metallic gear-wheels of this type over methods heretofore used; at the same time I have found by extensive tests that the finished product in the case of gear-wheels, is stronger and more durable than similar gear-wheels made by previous known methods. By my method I am enabled to utilize initially baled cotton or various wastes from cotton mills which represents the lowest initial cost for raw material. This constitutes one saving in cost accomplished by my invention. Another saving in cost results from the fact that the method is simple to carry out, effecting a decrease in both the labor and factory equipment required. In addition to the foregoing by my improved method I effect an additional saving in that the scrap material left from cutting the discs from the board-like sheets can be re-worked in the two beater picker whereby it results that all waste of material is eliminated.

What I claim as new and desire to secure by Letters Patent of the United States is:

1. The method of forming sheets of spinable textile material from which pieces for

use in the manufacture of gear wheels or the like may be cut, which comprises treating the textile material with lubricating oil, and then compressing it to form sheets.

5. The method of forming sheets of unwoven textile material from which pieces for use in the manufacture of gear wheels or the like may be cut, which comprises treating layers of textile fibers as they come from a picker with lubricating oil, placing the treated layers one on another, and then compressing them to form sheets.

10 3. The method of forming sheets of spinable textile material from which pieces for use in the manufacture of gear wheels or the like may be cut, which comprises treating the textile material with lubricating oil and then consolidating sheets of the material by the application of pressure and heat to form sheets.

15 4. The method of forming sheets of spinable textile material from which pieces for making gear wheels or the like may be cut, which comprises treating the textile material with lubricating oil and then passing it between rolls to compress it to form sheets.

20 5. The method of forming sheets of unwoven textile material from which pieces for use in the manufacture of gear wheels or the like may be cut, which comprises treating the unwoven textile material with lubricating oil and then compressing it to form sheets.

In witness whereof, I have hereunto set my hand this thirteenth day of April, 1928.

35 GUY O. SMALL.